

# United States Patent [19]

Sung et al.

[11] Patent Number: 4,808,335

[45] Date of Patent: Feb. 28, 1989

---

[54] OXIDATION AND CORROSION RESISTANT  
DIESEL ENGINE LUBRICANT

[75] Inventors: Rodney L. Sung, Fishkill; Benjamin  
H. Zoleski, Beacon; Ronald L.  
O'Rourke, Hyde Park, all of N.Y.

[73] Assignee: Texaco Inc., White Plains, N.Y.

[21] Appl. No.: 115,330

[22] Filed: Nov. 2, 1987

[51] Int. Cl.<sup>4</sup> ..... C10M 105/22

[52] U.S. Cl. ..... 252/47.5; 252/51.5 R;  
252/51.5 A

[58] Field of Search ..... 252/51.5 A, 51.5 R,  
252/47.5

## [56] References Cited

### U.S. PATENT DOCUMENTS

4,036,766 7/1977 Yamamoto ..... 252/51.5 A

4,087,386 5/1978 Dounchis ..... 252/32.5  
4,386,001 5/1983 Zoleski ..... 252/32.7  
4,536,307 8/1985 Horodysky ..... 252/51.5 A X  
4,711,735 12/1987 Gulley ..... 252/180 X

*Primary Examiner*—Jacqueline V. Howard

*Assistant Examiner*—James M. Hunter, Jr.

*Attorney, Agent, or Firm*—Robert A. Kulason; James J.  
O'Loughlin; Louis S. Sorell

## [57] ABSTRACT

An oxidation and corrosion resistant diesel engine lubricant composition, particularly useful in marine and railway diesel engines, comprises a major amount of a base hydrocarbon lubricating oil and from 0.1-5.0 weight percent of a reaction product additive which is the reaction product of an N-acyl sarcosine and a substituted or unsubstituted heterocyclic azole.

20 Claims, No Drawings

OXIDATION AND CORROSION RESISTANT  
DIESEL ENGINE LUBRICANT

BACKGROUND OF THE INVENTION

1. Field of the Invention

This invention relates to a diesel engine crankcase lubricating composition which exhibits improved resistance to corrosion and oxidation. More particularly, this invention relates to a novel corrosion and oxidation resistant diesel engine crankcase lubricating composition comprising a major amount of a hydrocarbon lubricating oil and a minor amount of the reaction product of an N-acyl sarcosine reactant and a substituted or unsubstituted heterocyclic azole reactant. The instant invention is particularly useful as a lubricant in large diesel engines such as marine and railway diesel engines.

2. Information Disclosure Statement

As is well known to those skilled in the art, lubricating oils must be characterized by resistance to oxidation and corrosion inhibition. Since the oils used as lubricants in the crankcases of large diesel engines, such as marine and railway diesel engines, are subject to unique conditions of operation, special attention must be directed to the potential problems which are to be encountered.

In addition, the advent of new, more fuel efficient railway diesel engines has put a greater demand on the oxidation resistance of railway diesel lubricants. Oxidized lubricants may lead to increased corrosive attack of engine metal surfaces; consequently, lubricants employed in newer railway diesel engines must be changed more frequently to prevent such corrosive attack.

In view of the above, diesel engine lubricant compositions have previously been specifically formulated containing anti-wear additives, demulsifying agents, oxidation and corrosion inhibitors and other additives. In particular, oxidation and corrosion-inhibited diesel engine lubricant formulations containing azole compound reaction products have been developed. For example:

Co-assigned U.S. patent application Ser. No. 115,491, filed Nov. 2, 1987 (D#78,549) (Sung et al.) discloses an oxidation and corrosion-resistant diesel engine lubricant composition comprising a major amount of a hydrocarbon lubricating oil and a minor amount of the reaction product prepared by first reacting a hydroxybenzoic acid with a polyoxyalkylene polyol to produce an ester, and thereafter reacting the esterification product with an aldehyde or ketone and a substituted or unsubstituted heterocyclic azole to form the final reaction product;

Co-assigned U.S. Pat. No. 4,705,642 (Sung et al.) discloses a haze, oxidation, and corrosion-resistant diesel engine lubricant composition which comprises a major amount of a hydrocarbon lubricating oil and a minor amount of the reaction product of an anhydride compound, a hydrocarbon-substituted mono primary amine or ether amine, and a nitrogen-containing heterocyclic azole or polyalkylene polyamine compound;

Co-assigned U.S. Pat. No. 4,464,276 (Sung et al.) describes the preparation of novel polyoxyalkylene polyamine-triazole complexes and their use in diesel lubricant compositions as antioxidants and corrosion-inhibitors; and

Co-assigned U.S. Pat. No. 4,285,823 (Sung et al.) discloses a diesel engine lubricant composition comprising a corrosion inhibitor which is the reaction product

of an N-alkyl-1,3 propane diamine, formaldehyde, and a 5-aminotetrazole.

The corrosion-inhibiting properties of N-acyl sarcosine reaction products in motor fuel compositions are also known to those skilled in the art. For example, the corrosion-inhibiting properties in alcohol and gasoline-alcohol compositions of the reaction product of (i) compounds including N-acyl sarcosines and (ii) aminotetrazoles are disclosed in co-assigned U.S. Pat. No. 4,445,907 (Sung). In addition, the corrosion-inhibiting properties in motor fuel compositions of the reaction product of (i) an N-acyl sarcosine reactant and (ii) a polyalkylene polyamine reactant are disclosed in co-assigned U.S. Pat. No. 4,305,731 (Sung et al.).

It is an object of this invention to provide a novel diesel engine lubricant composition. It is another object of this invention to provide a novel lubricant composition, suitable for use in large marine and railway diesel engines, characterized by its resistance to oxidation and corrosion. It is yet another object of this invention to provide a method of preparing such a diesel engine lubricant composition, as well as a method of inhibiting the oxidation of a diesel engine lubricant composition.

It is a feature of this invention that a diesel engine lubricant comprising a major amount of a hydrocarbon lubricating oil and a minor amount of the reaction product of an N-acyl sarcosine reactant and a substituted or unsubstituted heterocyclic azole reactant is characterized by its resistance to oxidation and corrosion. It is another feature of this invention that such a diesel engine lubricant composition is particularly suitable for use in large marine and railway diesel engines.

It is an advantage of this invention that the corrosion of diesel engine metal surfaces is reduced by employing this invention as a lubricant. It is another advantage of this invention that it may be changed less frequently than other conventional diesel engine lubricants.

SUMMARY OF THE INVENTION

The instant invention relates to a diesel engine crankcase lubricant composition which exhibits improved corrosion and oxidation resistance as compared with conventional diesel engine lubricant formulations. The novel lubricant composition of the instant invention comprises a major proportion of a hydrocarbon lubricating oil and from about 0.1 to 5.0 weight percent, preferably 0.5-2.0 weight percent (based on the lubricating oil) of the reaction product obtained by reacting, at a temperature range of 50° C.-200° C., preferably 60° C.-150° C., substantially equimolar amounts of:

(a) an N-acyl sarcosine reactant of the formula:



where R is a C<sub>8</sub>-C<sub>24</sub> alkyl radical, preferably a C<sub>12</sub>-C<sub>20</sub> alkyl radical, most preferably oleyl, and R' is H or a C<sub>1</sub>-C<sub>6</sub> alkyl radical, most preferably CH<sub>3</sub>; and

(b) a substituted or unsubstituted heterocyclic azole reactant, preferably selected from the group consisting of tolyltriazole, benzotriazole, aminotriazole, aminotetrazole, aminomercaptothiadiazole, and benzomercaptothiazole, most preferably 5-aminotriazole.

This invention is also directed to a method of preparing the above described diesel engine lubricating oil,

and to a method of inhibiting the oxidation of a diesel engine lubricating oil composition.

### DESCRIPTION OF THE PREFERRED EMBODIMENTS

The diesel lubricant compositions of the instant invention include lubricating oils which are employed in large diesel engines, particularly in the crankcases of large diesel engines such as are found in marine service, and in large railway diesel engines.

The novel corrosion and oxidation resistant diesel engine lubricating oil of the instant invention comprises a major amount of a base hydrocarbon lubricating oil and from 0.1 to 5.0 weight percent, preferably 0.5 to 2.0 weight percent of a corrosion and oxidation-inhibiting additive which is the reaction product of an N-acyl sarcosine reactant and a substituted or unsubstituted heterocyclic azole reactant.

The base hydrocarbon oil which may be employed to prepare the lubricating oil composition of the invention includes naphthenic base, paraffinic base and mixed base mineral oils, lubricating oil derived from coal products and synthetic oils, e.g. alkylene polymers such as polypropylene and polyisobutylene of a molecular weight of between about 250 and 2500. In the case of marine diesel engine lubricants, the preferred lubricant is typically a hydrocarbon lubricating oil having a Total Base Number (TBN) of 3-8, say 6 made up for example by blending a paraffinic Solvent Neutral Oil (SNO-20) having a VI of ca 92 and a viscosity of 47-53 CSt at 40° C. and 6.65-7.15 at 100° C. with a paraffinic Solvent Neutral Oil (SNO-50) having a VI of ca 93 and a viscosity of 158-180 CSt at 40° C. and 15.3-16.4 at 100° C. In the case of railway diesel engine lubricants, the preferred lubricant is typically a mixture of a paraffinic mineral oil of a viscosity of 5.5-10.0, say 8.5 CSt at 100° C., a paraffinic mineral oil of a viscosity of 8.0-15.0, say 14.5 CSt at 100° C., and a naphthenic pale oil of a viscosity of 8.0-15.0, say 14.2 CSt at 100° C.

Typically, the lubricant composition of the instant invention may contain minor amounts of additional additives. Table I sets forth illustrative additives which may be employed in admixture with the instant invention when it is used as a marine diesel engine lubricant.

TABLE I

| Additive Function   | Broad Range (wt. %) | Illustrative Additive                       |
|---------------------|---------------------|---------------------------------------------|
| Anti-wear Agent     | 0.1-1               | Zinc dialkyl dithiophosphate                |
| Oxidation Inhibitor | 0.1-1               | alkylated diphenyl amine                    |
| Demulsifying Agents | 50-200 ppm          | dimethyl polysiloxane (a silicone)          |
| Detergent           | 1-5                 | Overbased sulfurized calcium alkylphenolate |
| Anti-Rust Agent     | 0.1-5               | Ethoxylated nonyl phenol                    |

When the lubricant composition of the instant invention is used as a railway diesel engine lubricant, additional additives or additive packages may also be employed. An illustrative example of an additive concentrate package (commercially available from Chevron Chemical Company as ORONITE OLOA 2939) which may be employed in admixture with the lubricant composition of the instant invention is set forth in Table II.

TABLE II

| Additive                                              | Typical Concentration (wt. %)* |
|-------------------------------------------------------|--------------------------------|
| Overbased mixed calcium petroleum sulfonate/phenolate | 45                             |
| Polyisobutylene                                       | 10                             |
| succinimide/amide                                     | 1.5                            |
| Polyisobutylene                                       | 1.5                            |
| Paraffinic Mineral Oil                                | 43                             |
| Chloroparaffin                                        | 0.5                            |

\*Wt. % concentration based on total weight of additive concentrate package.

The N-acyl sarcosine reactant is of the formula:



where R is a C<sub>8</sub>-C<sub>24</sub>, preferably a C<sub>12</sub>-C<sub>20</sub> alkyl radical, more preferably an alkyl radical selected from the group consisting of oleyl, coco, lauryl, stearyl, and tallow, most preferably oleyl, and R' is H or a C<sub>1</sub>-C<sub>6</sub> alkyl radical, most preferably CH<sub>3</sub>.

Examples of N-acyl sarcosine reactants suitable for use are those sold under the SARKOSYL trademark by the Ciba-Geigy Company, and they include SARKOSYL-O (oleoyl sarcosine) having a molecular weight in the range of about 345-360, SARKOSYL-L (lauryl sarcosine), having a molecular weight in the range of about 270-285, SARKOSYL-LC (cocoyl sarcosine), having a molecular weight in the range of about 285-300, SARKOSYL-S (stearoyl sarcosine), having a molecular weight in the range of about 330-345, and SARKOSYL-T (tallow sarcosine), having a molecular weight in the range of about 360-370. Oleoyl sarcosine is particularly preferred for use as the N-acyl sarcosine reactant.

The heterocyclic azole reactant may be any substituted or unsubstituted heterocyclic azole, but preferably is selected from the group consisting of tolyltriazole (hereinafter referred to as TTZ), benzotriazole (hereinafter referred to as BTZ), aminotriazole (hereinafter referred to as ATZ), aminotetrazole (hereinafter referred to as ATTZ), aminomercaptothiadiazole (hereinafter referred to as AMTZ), and benzomercaptothiazole (hereinafter referred to as BMTZ).

If an aminotriazole reactant is employed, it preferably will be a 3-, 4-, or 5-aminotriazole (hereinafter referred to as 3-ATZ, 4-ATZ, or 5-ATZ, respectively), including those bearing inert substituents, typified by hydrocarbon or alkoxy groups, which do not react in the instant invention. The most preferred aminotriazole reactant is 5-ATZ. If an aminotetrazole reactant is employed, it preferably will be a 4- or 5-aminotetrazole (hereinafter referred to as 4-ATTZ or 5-ATTZ, respectively), again including those bearing inert substituents, typified by hydrocarbon or alkoxy groups which do not react in the instant invention. If an aminomercaptothiadiazole reactant is employed, it preferably will be a 5-aminomercaptothiadiazole. The most preferred hydrocarbyl azole reactant for use in the instant invention is 5-ATZ.

In a preferred mode of preparing the reaction product, the N-acyl sarcosine reactant is first dissolved in an excess of a non-alcohol solvent. Typical solvents which may be employed include hydrocarbons including hep-

tane, octane, toluene, xylene, gasoline, etc. Xylene is particularly preferred for use as a solvent. A substantially equimolar amount of the heterocyclic azole reactant is thereafter added, and the reaction mixture is refluxed at a temperature range of 50° C.-200° C., preferably 60° C.-150° C., until such time as no more water can be removed from the reaction mixture. The reaction may generally be completed in from about 0.1-10 hours, although longer time may be required for large quantities. After the water is removed from the system, the reaction product may be filtered and stripped of the solvent using conventional means, or left in admixture with some or all of the solvent to facilitate addition of the reaction product to the base lubricant oil.

The following examples illustrate the preferred method of preparing the reaction product. It will be understood that the following examples are merely illustrative, and are not meant to limit the invention in any way. In the examples, all parts are parts by weight unless otherwise specified.

#### EXAMPLE 1

In a preferred mode of preparing the reaction product compound of the instant invention, 87.3 parts of oleoyl sarcosine (SARKOSYL-O), 21 parts of 5-ATZ, and 173 parts of xylene were reacted at the reflux temperature of xylene and azeotroped until no more water could be removed from the system. The reaction mixture was cooled, filtered and stripped of remaining solvent under a vacuum.

#### EXAMPLE 2

A reaction product compound is prepared by reacting 175 parts of cocoyl sarcosine (SARKOSYL-LC), 42.5 parts of 5-ATTZ, and 4 parts of crystallite (a hydrocarbon solvent having a boiling range of 300° F.-550° F.). The mixture is refluxed at 175° C. until such time as no more water can be removed from the system. The reaction mixture is thereafter cooled, filtered, and stripped of remaining solvent under a vacuum.

The reaction product additive may be added to the base lubricating oil in minor, effective, corrosion inhibiting amounts of about 0.1-5.0 wt. %. Lesser quantities may be employed, but the degree of improvement so obtained may be lessened thereby. Larger amounts may be employed, but no significant additional improvement is thereby attained. Preferably the effective amount is about 0.5-2.0 wt. %, say about 1.0 wt. % based on the lubricating oil. The reaction product compound may be added separately or as a component of an additive package which contains other additives.

Presence of the above-described reaction product compound in a diesel engine lubricating oil such as a railway diesel engine lubricant is found to be particularly advantageous in controlling the degradation characteristics of the lubricant. Degradation of the lubricant often leads to higher acid concentrations within the lubricant, which may in turn lead to corrosive attack of metallic engine surfaces.

The ARCO Railroad Oil Oxidation Test (ARCO 60 Test) was employed to determine the degradation characteristics of lubricant compositions of the instant invention. The ARCO Test is intended for the determination of the oxidation and corrosion characteristics of diesel engine lubricants, is especially useful as a screening test for railway diesel engine lubricants.

The ARCO Test method involves bubbling oxygen at a rate of 5 liters/hr. through 300 gm of test oil held at

300° F. in the presence of three metal coupons, one each made of copper, lead, and steel. At the end of the Test, the total weight change of the coupons is measured, thereby determining the corrosion characteristics of the test oil vis-a-vis the metal coupons. The detailed procedure of the ARCO Test is set forth below.

Three square metal coupons are cut from metal sheets, as follows:

| COU-<br>PON | MATERIAL            | DIMENSIONS |   |      | WEIGHT.<br>gm<br>APPROX. |       |
|-------------|---------------------|------------|---|------|--------------------------|-------|
|             |                     | mm         | × | mm   |                          |       |
| Copper      | Electrolytic Copper | 25.4       | × | 25.4 | 3.12                     | 17-18 |
| Steel       | Mild Carbon Steel   | 25.4       | × | 25.4 | 3.07                     | 15-16 |
| Lead        | Chemical Grade Lead | 25.4       | × | 25.4 | 1.52                     | 11-12 |

Two 2.38-mm holes are drilled in each coupon, and the coupons are polished with fine emery cloth and steel wool to obtain a clean, smooth surface, then washed with acetone, dried, and tared. Using clean cotton cord, the coupons are tied together as a hollow prism which stands in an oxidation cell assembly. The oxidation cell includes a test tube, an oxygen inlet tube and a condenser, and is the same cell as used in ASTM Method D-943 "Oxidation Characteristics of Inhibited Steam Turbine Oils" except that no cooling water is used for the condenser.

After placing the coupons into the oxidation cell, the cell is filled with 300 gm of the oil to be tested. The cell is then placed in an oil bath which has been previously adjusted to a temperature of 300±2° F., and heated for 48 hours. Oxygen at a flow rate of 5±0.2 liters/hr. is constantly contacted with the test oil. At the end of 48 hours, the oxygen flow is stopped, and the cell is taken out of the bath and allowed to cool to room temperature.

The coupons are then removed from the cell, washed with a 50/50 blend of toluene and acetone, and allowed to dry. The coupons are thereafter weighed to determine weight changes due to oil oxidation of the metal surfaces. The weight changes of the coupons are reported as the total weight loss of all three coupons. A large weight loss indicates a very corrosive oil which can lead to corrosive attack of engine metal surfaces. In addition, the viscosities of the test oil before and after the Test are measured to determine the effect of oxidation on oil viscosity. The greater the percentage increase in viscosity due to oxidation, the greater the degree of oil degradation which has occurred.

The following examples and ARCO Test results further illustrate the superiority of the instant invention as a diesel engine lubricant, particularly as a railway diesel engine lubricant.

#### EXAMPLE 3

In this control example, a standard railway diesel engine lubricant was formulated containing the following components:

| Component                                                    | wt. % |
|--------------------------------------------------------------|-------|
| (i) Paraffinic mineral oil of viscosity 8.46 CSt at 100° C.  | 19.12 |
| (ii) Paraffinic mineral oil of viscosity 14.5 CSt at 100° C. | 22.48 |
| (iii) Naphthenic pale oil of viscosity 14.2 CSt at 100° C.   | 43.76 |
| (iv) ORONITE OLOA 2939 brand                                 | 14.64 |

-continued

| Component         | wt. % |
|-------------------|-------|
| additive package* |       |

\*See Table II

This formulation is representative of conventional railway diesel engine crankcase lubricants. It was tested via the ARCO Test and found to have a total coupon weight loss of 0.2208 gm and a viscosity increase of 14.7%.

## EXAMPLE 4

A lubricant formulation was made up containing 99 wt. % of the base lubricant of Example 3 and 1.0 wt. % of the reaction product of Example 1. This formulation is representative of lubricant formulations of the instant invention. It was tested via the ARCO Test and found to have a total coupon weight loss of 0.0830 gm and a viscosity increase of 11.3%.

As demonstrated by a comparison of the ARCO Test results for Examples 3 and 4, a composition of the instant invention formulated for use as a railway diesel engine lubricant (Example 4) exhibited less degradation after exposure to the test conditions of the ARCO Test than a conventional railway diesel engine lubricant formulation (Example 3). Example 4 showed both lower viscosity increase (hence less oxidation) and lower total coupon weight loss (hence less corrosive attack of metal surfaces) than the conventional lubricant of Example 3; therefore the instant invention as exemplified by Example 4 is superior to a conventional diesel lubricant as exemplified by Example 3 in terms of both oxidation and corrosion resistance.

Although this invention has been illustrated by reference to specific embodiments, it will be apparent to those skilled in the art that various changes and modifications may be made which clearly fall within the scope of this invention. For example, reaction product compositions of the instant invention may also be useful as corrosion inhibitors in other types of compositions such as motor fuels, alcohols, metal working fluids, and the like.

We claim:

1. A diesel engine lubricating oil composition comprising a major amount of a hydrocarbon lubricating oil and from 0.1-5.0 weight percent of the reaction product obtained by reacting at a temperature range of 50° C.-200° C. substantially equimolar amounts of:

(a) an N-acyl sarcosine reactant of the formula:



wherein R is a C<sub>8</sub>-C<sub>24</sub> alkyl radical and R' is H or a C<sub>1</sub>-C<sub>6</sub> alkyl radical; and

(b) a substituted or unsubstituted heterocyclic azole reactant.

2. A lubricating oil composition according to claim 1, where R is a C<sub>12</sub>-C<sub>20</sub> alkyl radical, and R' is a methyl radical.

3. A lubricating oil composition according to claim 1, where R is an alkyl radical selected from the group consisting of oleyl, coco, lauryl, tallow, and stearyl.

4. A lubricating oil composition according to claim 1, where said N-acyl sarcosine reactant is selected from

the group consisting of oleyl, lauroyl, cocoyl, stearoyl, and tallow sarcosine.

5. A lubricating oil composition according to claim 1, where said heterocyclic azole reactant is an aminotriazole.

6. A lubricating oil composition according to claim 5, where said aminotriazole is 5-aminotriazole.

7. A lubricating oil composition according to claim 1, where said heterocyclic azole reactant is an aminotetrazole.

8. A lubricating oil composition according to claim 7, where said aminotetrazole is selected from the group consisting of 4- and 5-aminotetrazole.

9. A lubricating oil composition according to claim 1, where said heterocyclic azole reactant is an aminomercaptothiadiazole.

10. A lubricating oil composition according to claim 9, where said aminomercaptothiadiazole is a 5-aminomercaptothiadiazole.

11. A lubricating oil composition according to claim 1, where said heterocyclic azole reactant is a benzomercaptothiazole.

12. A lubricating oil composition according to claim 1, where said heterocyclic azole reactant is benzotriazole.

13. A lubricating oil composition according to claim 1, where said heterocyclic azole reactant is tolyl-triazole.

14. A diesel engine lubricating oil composition comprising a major amount of a hydrocarbon lubricating oil and from 0.1-5.0 weight percent of the reaction product obtained by reacting at a temperature range of 50° C.-200° C. substantially equimolar amounts of:

(a) an N-acyl sarcosine reactant of the formula:



(b) 5-aminotriazole.

15. A lubricating oil composition as in any one of the claims 1-14, in which said composition comprises a major amount of a hydrocarbon lubricating oil and from 0.5-2.0 weight percent of said reaction product.

16. A method of preparing a diesel engine lubricating oil composition which comprises adding to a major portion of a hydrocarbon lubricating oil 0.1-5.0 weight percent of a reaction product prepared by reacting at a temperature range of 50° C.-200° C. substantially equimolar amounts of:

(a) an N-acyl sarcosine reactant of the formula:



wherein R is a C<sub>8</sub>-C<sub>24</sub> alkyl radical and R' is H or a C<sub>1</sub>-C<sub>6</sub> alkyl radical; and

(b) a substituted or unsubstituted heterocyclic azole reactant.

17. A method of preparing a diesel engine lubricating oil composition which comprises adding to a major portion of a hydrocarbon lubricating oil 0.1-5.0 weight percent of a reaction product prepared by reacting at a

temperature range of 50° C.-200° C. substantially equimolar amounts of:

(a) an N-acyl sarcosine reactant of the formula:



(b) 5-aminotriazole.

18. A method of inhibiting the oxidation of a diesel engine lubricating oil composition which comprises adding to a major portion of a hydrocarbon lubricating oil 0.5-5.0 weight percent of a reaction product prepared by reacting at a temperature range of 50° C.-200° C. substantially equimolar amounts of:

(a) an N-acyl sarcosine reactant of the formula:

5



wherein R is a C<sub>8</sub>-C<sub>24</sub> alkyl radical and R' is H or a C<sub>1</sub>-C<sub>6</sub> alkyl radical; and

10 (b) a substituted or unsubstituted heterocyclic azole reactant.

19. A method of inhibiting the oxidation of a diesel engine lubricating oil composition which comprises adding to a major portion of a hydrocarbon lubricating oil 0.5-5.0 weight percent of a reaction product prepared by reacting at a temperature range of 50° C.-200° C. substantially equimolar amounts of:

(a) an N-acyl sarcosine reactant of the formula:

20



(b) 5-aminotriazole.

25 20. The method of any of claims 16-19, in which 0.5-2.0 weight percent of said reaction product is added to said hydrocarbon lubricating oil.

\* \* \* \* \*

30

35

40

45

50

55

60

65